



US005618401A

**United States Patent** [19]**Nomura et al.**[11] **Patent Number:** **5,618,401**[45] **Date of Patent:** **Apr. 8, 1997**

[54] **INNER-SHIELD MATERIAL TO BE ATTACHED INSIDE A COLOR CATHODE RAY TUBE AND MANUFACTURING METHOD THEREOF**

[75] Inventors: **Giichiro Nomura; Osamu Yubuta**, both of Kudamatsu, Japan

[73] Assignee: **Toyo Kohan Co., Ltd.**, Tokyo, Japan

[21] Appl. No.: **378,873**

[22] Filed: **Jan. 24, 1995**

**Related U.S. Application Data**

[60] Continuation of Ser. No. 197,273, Feb. 16, 1994, abandoned, which is a division of Ser. No. 91,683, Jul. 15, 1993, abandoned.

[30] **Foreign Application Priority Data**

Jul. 16, 1992 [JP] Japan ..... 4-213309

[51] **Int. Cl.<sup>6</sup>** ..... **C25D 5/02; C25D 7/06; C25D 5/34; C21D 8/12**

[52] **U.S. Cl.** ..... **205/130; 205/138; 205/152; 205/206; 205/207; 205/217; 205/227; 205/271; 148/530; 148/534**

[58] **Field of Search** ..... 205/130, 137, 205/138, 152, 206, 207, 217, 224, 227, 271; 148/530, 534

[56] **References Cited**

**U.S. PATENT DOCUMENTS**

2,115,750 5/1938 Rubin et al. ..... 204/14

|           |         |                 |       |           |
|-----------|---------|-----------------|-------|-----------|
| 3,095,361 | 2/1961  | Stone           | ..... | 205/207   |
| 4,385,256 | 5/1983  | Tokita et al.   | ..... | 313/407   |
| 4,775,599 | 10/1988 | Matsuoka et al. | ..... | 428/600   |
| 5,094,920 | 3/1992  | Shiozaki et al. | ..... | 428/472.1 |
| 5,252,151 | 10/1993 | Inoue et al.    | ..... | 148/541   |

**FOREIGN PATENT DOCUMENTS**

|           |         |       |   |
|-----------|---------|-------|---|
| 59-53682  | 3/1984  | Japan | . |
| 61-3472   | 1/1986  | Japan | . |
| 61-235594 | 10/1986 | Japan | . |
| 61-15393  | 1/1989  | Japan | . |
| 3166388   | 7/1991  | Japan | . |

**OTHER PUBLICATIONS**

Merriman, a Dictionary of Metallurgy (1958), p. 278.

*Primary Examiner*—Donald R. Valentine

*Assistant Examiner*—Edna Wong

*Attorney, Agent, or Firm*—Browdy and Neimark

[57] **ABSTRACT**

A method of making, for cathode ray tubes and the like, an inner shield material that has superior magnetic characteristics and rust resistance. The method does not require conventional blackening processes. Sheet steel or strip is nickel-plated with a nickel-iron diffusion layer and then annealed. The annealing improves the magnetic characteristics. The sheet is cold-rolled prior to annealing to provide a roughened surface, which decreases the chances of sticking during the annealing process. In one embodiment the sheet is pickled, cold-rolled, annealed, cold rolled again, nickel plated, and then annealed again. Annealing between the first and second cold-rolling operations improves the magnetic characteristics.

**3 Claims, No Drawings**

INNER-SHIELD MATERIAL TO BE  
ATTACHED INSIDE A COLOR CATHODE  
RAY TUBE AND MANUFACTURING  
METHOD THEREOF

This application is a continuation of application Ser. No. 08/197,273, filed Feb. 16, 1994 now abandoned which is a divisional of application Ser. No. 08/091,683 filed Jul. 15, 1993 now abandoned.

BACKGROUND OF THE INVENTION

1. Field of the Invention

The present invention relates to an inner-shield material to be attached inside a color cathode ray tube and its manufacturing method, especially to the manufacturing method for the inner-shield material having superior magnetic characteristics and rust protection or corrosion resistance that eliminates a blackening process in its manufacturing method.

The magnetic shield material for a color cathode ray tube is attached to an outer or inner side of the color cathode ray tube to prevent electron beams from being deflecting by terrestrial magnetism. The magnetic shield material attached inside the tube is referred to as an inner shield material, while that outside the tube is referred to as an outer-shield material. In addition to such magnetic characteristics as higher permeability and lower coercive force, the characteristics on thermal radiation and rust protection are required for the magnetic-shield material.

For this purpose, for example, in Japanese Patent Publication No. 1894 of 1989 (hereafter referred to as "the former reference"), the use of Ni- or Cr-plated steel sheet or strip as inner-shield materials and the technique for blackening the surface of the plated steel sheet or strips in the heat treatment on the color cathode ray tube manufacturing process have been disclosed. However, this technique is only for manufacturing color cathode ray tubes, it could not be extended to manufacturing inner-shield materials. On the other hand, TOKU KAI HEI 2 (Japanese Unexamined Patent Publication 1990) 228466 (hereafter referred to as "the latter reference") disclosed a technique for forming a blackened film or coat with FeO contained as its main constituent on the surface of a thin steel sheet or strip using an oxidizing gas and a non-oxidizing gas in a continuous annealing line in an inner-shield material manufacturing process. The latter reference mentioned that this technique could eliminate the blackening process in the manufacture of color cathode ray tube.

The former reference suggests that the use of Ni- or Cr-plated steel sheet or strips may eliminate the blackening process which has been necessary for conventional non-plated steel sheet or strip. In effect, some manufacturers use ultra-thin Cr-plated steel sheet or strips as an inner-shield material.

Usually, however, the ultra-thin Cr-plated steel sheet or strips described in the former reference are produced through a sequential process of annealing, skin pass rolling, and plating. Thus, ultra-thin Cr-plated steel sheet or strip have the disadvantage of inferior magnetic characteristics inasmuch as the grains of the annealed steel sheet or strip are distorted by the skin pass rolling. It was found that these magnetic characteristics by themselves could be improved by modifying the manufacturing process to use the sequential processes of plating and annealing. However, nobody

has used this process because of some difficulties in the plating step following annealing, as discussed below.

That is to say, the material, prior to being subjected to the plating process, has been softened through the annealing process, and moreover, its thickness is very thin (in general, steel sheet or strips with a thickness of 0.15 mm are used).

Thus, the material cannot be passed through the plating process because of the so-called "wrinkle" on its surface. Or even when it may pass through the process, the material is so deformed that it is unusable as an inner-shield material.

On the other hand, the method described in the latter reference is considered to be better than that the method described in the former reference with respect to providing good magnetic characteristics.

The blackening is executed in the continuous annealing furnace in accordance with the following steps.

① Heating process

Forming  $Fe_3O_4$  in an oxidizing gas

② Soaking process

Transforming  $Fe_3O_4$  into FeO in a non-oxidizing gas

③ Cooling process

Rapidly cooling the steel sheet or strip in the non-oxidizing gas atmosphere to form the blackening film containing FeO as the principal constituent

This method is a new technique for improving the blackening film's adhesion by transforming the  $Fe_3O_4$  having inferior adhesion to the material into FeO, which can eliminate the blackening process in color cathode ray tube manufacturers.

The latter reference, however, suggests the following:

a) The heating pattern and the gas atmosphere should be strictly controlled to form a blackening film which can withstand to the press forming process.

b) The blackening film containing FeO as a principal constituent should be formed on the surface of the material under strictly controlled conditions.

These suggestions mean that in the method of the latter reference, it is likely that  $Fe_3O_4$  with inferior adhesion may be occasionally formed.

Thus, in the latter reference, some manufacturing and quality assurance problems exist because  $Fe_3O_4$  with inferior adhesion might be produced if strict control over manufacturing conditions is not maintained.

The object of the present invention is to provide both an inner-shield material and with superior magnetic characteristics and rust protection and a method for its manufacture which does not require a conventional blackening process.

Another object of the present invention is to provide an inner-shield manufacturing method, by which steel sheet or strip passing is made smooth in the plating process and the Ni-plated steel sheet or strip is prevented from sticking in the annealing process.

SUMMARY OF THE INVENTION

To achieve the above objects, the present invention provides an inner-shield material (aluminum-killed, cold rolled steel sheet or strip with a specified surface roughness), which has a nickel-iron diffusion layer on at least one side and a nickel layer over the nickel-iron diffusion layer.

Further, the present invention provides a method for manufacturing an inner-shield material which is provided by processing low-carbon, aluminum-killed steel strip sequentially through the steps of acid pickling, cold-rolling, Ni-plating and annealing.

Thus, this annealing of the Ni-plated steel sheet or strip adjusts the grains of the material and greatly improves the magnetic characteristics of the inner-shield material.

In addition, cold-rolling the steel sheet or strip before Ni-plating facilitates the steel sheet or strip passing in the Ni-plating process and prevents the Ni-plated steel sheet or strip from sticking in the annealing process.

According to the present invention, another method for manufacturing the inner-shield material is provided by passing the steel sheet or strip sequentially through the processes of acid pickling, primary cold-rolling, annealing, secondary cold-rolling, Ni-plating, and re-annealing.

Thus, annealing between the primary and secondary cold-rolling steps greatly improves the magnetic characteristics of the material.

#### DESCRIPTION OF THE PREFERRED EMBODIMENTS

The manufacturing method used for inner shield materials involves the step of cold-rolling aluminum-killed, cold-rolled steel sheet or strip with the surface roughness of 0.2–2.0  $\mu\text{m}$  Ra, the step of surface-treatment for depositing a nickel layer with a thickness of 0.1–5.0  $\mu\text{m}$  on at least one side of said steel sheet or strip, and the step of annealing said surface-treated steel sheet or strip.

The details of preferred embodiments of the method of the present invention are described hereinafter.

##### 1. Acid Pickling

Before the cold rolling process, the base steel is preferably processed to an acid pickling in order to eliminate hot band scales in the acid solution. In this case, sulfuric or hydrochloric acid is preferably used.

Note that to facilitate the elimination of scales, a method for cracking scales on the surface of the hot band using any means such as a scale breaker located at the entrance of the line can be used simultaneously.

##### 2. Cold-Rolling Process

The hot band are continuously cold-rolled to approximately the given thickness by a continuous cold rolling mill.

The dull surface roll can be used to dull the surfaces of the steel sheet or strip to adjust their surface roughness during cold-rolling. The transcription rate from the roll to the strip is about 10–20%. In this case, palm oil is used as a rolling oil. In this process, the steel sheet or strip should be checked for steel thickness, surface defects, and shape. Whale oil or tallow based synthetic oil can be also used as the rolling oil.

After rolling, the steel sheet or strip are electrolytically degreased in a solution such as sodium orthosilicate in order to remove the rolling oil.

To enhance the degreasing ability of the solution, some surfactant can be added.

Note that to increase the degreasing ability in the cleaning process the steel sheet or strip are preferably used as an electrode in the bath. In this case,  $\text{H}_2$  and  $\text{O}_2$  generated on the steel strip surface act to separate the rolling oil mechanically from the steel surface.

##### 3. Skin Pass Rolling Process

According to the method claimed in the present invention, the surface roughness can be adjusted in the cold-rolling step, or in the skin pass rolling step following cold-rolling.

Generally, in the surface treatment of the steel sheet or strip manufacturing process, annealing is usually followed by skin pass rolling to prevent from fluting, stretcher strain, to flat the shapes of the strip, and to print surfaces roughness.

In general, the steel sheet or strip is cold-rolled a little at the rolling reduction of approximately 0.5–3.0% in the drying process without using a rolling oil.

However, according to the method claimed in the present invention, the steel sheet or strip is skin pass-rolled after the steps of cold-rolling and cleaning.

in addition, dulling the surfaces of the steel sheet or strip prevents the strip from sticking and prevents flaws from appearing on the surfaces during annealing.

##### 4. Ni-Plating Process

The surface of the steel sheet or strip is cleaned and activated through the steps of degreasing and acid cleaning, and then Ni-plated.

In the present invention, Ni-plating is applied because of its superior rust protection and its characteristic of not affecting the intrinsic magnetic properties of the steel sheet or strip.

In addition, the Ni-plated steel sheet or strip has a benefit in that the blackening process in cathode ray picture tube manufacturer can be eliminated.

In Ni-plating, a nickel-sulfate bath (so-called Watt bath) is usually used. Other ordinary Ni-plating baths, however, such as a nickel chloride bath or sulfamime acid bath, etc. can also be used.

Note that according to the present invention, the thickness of the Ni-plating is thinner than those applied in conventional nickel plating. A nickel anode is a nickel pellet contained in a titanic basket wrapped in a synthetic-fiber bag. Slime or sludge is thus prevented from being in suspension.

Any suspension in the plating bath causes a projection on the surface or pinholes in the plating layer as a result of co-deposition. To eliminate such a suspension, the plating solution is always circulated through a filter.

To achieve higher corrosion resistance, a thicker layer of Ni-plating is usually applied to the surface of the steel sheet or strip.

However, the means outlined above enables a thinner layer of Ni-plating to provide high corrosion resistance.

Thus, a Ni-plating layer with a thickness between 0.1–5.0  $\mu\text{m}$  can be applied. Note that a thickness greater than 5.0  $\mu\text{m}$  is considered to be uneconomical.

##### 5. Annealing Step

In the annealing step, the Ni-plated steel sheet or strip are box-annealed to facilitate re-crystallization and grain growth of the steel sheet or strip, and to improve the magnetic characteristics.

$\text{H}_2$  and  $\text{N}_2$  gases are flowed into the furnace to prevent Ni plating layer from discoloration as a result of oxidization.

The steel sheet or strip should be annealed in the furnace at 580° C.–620° C. for five to eight hours. In this process the rolling texture made in the cold rolling step is recrystallized and the grains are grown. This heat treatment achieves higher maximum magnetic permeability  $\mu\text{m}$ , and a lower coercive force  $\text{Hc}$ .

In the process, moreover, the recrystallized grains and the Fe-Ni diffusion layer are formed in the Ni plating layer to enhance toughness, adhesion, and corrosion resistance.

Note that to avoid sticking between steel sheet or strip to each other during the annealing process, a proper annealing temperature and length of time are selected. Moreover the surface of the steel sheet or strip is dulled by cold-rolling or skin pass rolling, and the coiling tension is adjusted.

The third aspect of the present invention is basically similar to the second aspect of the present invention with the exception that the steel sheet or strip is annealed, and is re-annealed after the Ni-plating process.

The inner-shield material is thus produced through the sequential steps of acid pickling, primary cold-rolling, annealing, secondary cold-rolling, Ni-plating, and re-annealing.

Only those points of difference are described below.  
(1) Primary Cold-Rolling

The primary cold-rolling is generally similar to said cold-rolling in the second aspect of the present invention. Note that the thickness of the produced steel sheet or strip may be 20-50% thicker compared with the thickness in the second aspect of the present invention.

(2) Annealing Step

In the embodiment in the third aspect of the present invention, the steel sheet or strip is annealed between the primary cold-rolling step and second cold rolling step. This annealing step is closely related to the post-process of secondary cold-rolling, and if necessary, to skin pass rolling.

Pre-annealing before the secondary cold-rolling step thus reduces rolling reduction substantially to grow larger grains during re-annealing and to enhance the magnetic characteristics of the material.

(3) Secondary Cold-Rolling

This process is basically similar to the second aspect of the invention except that the steel sheet or strip is rolled into the final thickness. However, care should be taken of the shape and thickness of the steel sheet or strip during cold-rolling, because these properties affect product quality directly.

(4) Re-Annealing

In the third aspect of the present invention, the steel sheet or strip is re-annealed. In the second aspect of the present invention, 2.3 mm hot band is cold-rolled to 0.15 mm thickness. In this case, 93.5% of the higher rolling reduction is applied.

The higher rolling reduction causes small grains to be formed after annealing and inferior magnetic characteristics.

In the third aspect of the present invention, the annealing and secondary cold-rolling steps are added to reduce the final rolling reduction to 20-50%. This lower rolling reduction causes larger grains to be formed after re-annealing.

Compared with the second aspect of the present invention, the re-annealing and secondary cold rolling steps are added to this third aspect of the present invention.

These processes make the lower cold reduction possible in the secondary cold-rolling step that precedes the re-annealing step and results in larger grains of the final product following the re-annealing step.

Note that the annealing furnace and gas atmosphere are the same as those in the second aspect of the present invention.

EXAMPLE

(1) Composition

The inner-shield material has been produced through the processes outlined below using a low-carbon aluminum-killed steel containing the compositions shown in Table 1.

TABLE 1

| Composition<br>(wt %) | C      | Si    | S     | Mn   | P     |
|-----------------------|--------|-------|-------|------|-------|
| Example               | 0.0045 | 0.005 | 0.005 | 0.24 | 0.013 |

(2) Manufacturing process

(Acid Pickling)

Hot band scales were removed in hot sulfuric acid. To facilitate the scale-removing, scales on the surfaces was cracked using a scale breaker at the entrance of the pickling line.

(Cold-Rolling)

2.3 mm thick hot band steel sheet or strip was cold-rolled into the thickness of 0.15 mm using continuous cold rolling mill.

Palm oil was used as the rolling oil and care was taken regard to steel thickness, surface defects and shape.  
(Cleaning)

To remove the rolling oil, the rolled-steel sheet or strip was electrolytically degreased in a bath such as the sodium orthosilicate solution. The temperature of the bath was 80° C.-100° C. A surfactant was added to the bath to enhance its degreasing ability.  
(Skin-Pass Rolling)

The steel sheet or strip with different surface roughness was produced through the skin-pass rolling step at an approximate 0.5% rolling reduction. The results are listed in Tables 2 and 3.

TABLE 2

| Sample<br>No.  | Surface<br>roughness<br>Ra (μm) | Sticking<br>in<br>annealing | Ni plating        |                         |            |            | Magnetic characteristics |                    |  |
|----------------|---------------------------------|-----------------------------|-------------------|-------------------------|------------|------------|--------------------------|--------------------|--|
|                |                                 |                             | thickness<br>(μm) | Corrosion<br>resistance | Br<br>(KG) | Hc<br>(Oe) | permea-<br>bility        | max.<br>evaluation |  |
| <u>Example</u> |                                 |                             |                   |                         |            |            |                          |                    |  |
| 1              | 0.21                            | ○                           | 0.42              | ○                       | 12.1       | 1.29       | 4215                     | ○                  |  |
| 2              | 0.28                            | ○                           | 1.00              | ○                       | 12.5       | 1.31       | 4307                     | ○                  |  |
| 3              | 0.42                            | ○                           | 0.10              | ○                       | 12.9       | 1.34       | 4316                     | ○                  |  |
| 4              | 0.44                            | ○                           | 0.20              | ○                       | 12.6       | 1.30       | 4382                     | ○                  |  |
| 5              | 0.47                            | ○                           | 2.50              | ○                       | 12.0       | 1.34       | 4022                     | ○                  |  |
| 6              | 0.56                            | ○                           | 5.00              | ○                       | 12.1       | 1.33       | 4271                     | ○                  |  |

TABLE 3

| Surface | Sticking | Ni plating | max. |
|---------|----------|------------|------|
|         |          |            |      |



TABLE 4-continued

| Sample No. | Annealing Temp. (°C.) | Surface roughness Ra (μm) | Sticking in annealing | Ni plating     |                      | Magnetic characteristics |         |                              |
|------------|-----------------------|---------------------------|-----------------------|----------------|----------------------|--------------------------|---------|------------------------------|
|            |                       |                           |                       | thickness (μm) | Corrosion resistance | Br (KG)                  | Hc (Oe) | permeability max. evaluation |
| 8          | 680                   | 2.06                      | ○                     | 0.37           | ◎                    | 10.3                     | 0.97    | 4980 ◎                       |

What we claimed is:

1. A manufacturing method used for the manufacture of inner-shield materials of a color cathode ray tube, comprising the steps of:

cold-rolling a cold-rolled steel sheet or strip to produce a surface roughness of 0.2–2.0 μm Ra,

electro-depositing a nickel layer with a thickness of 0.1–5.0 μm at least on one side of said steel sheet or strip,

annealing said surface-treated sheet or strip; and inserting the annealed steel sheet or strip into the cathode ray tube for magnetic shielding.

2. A manufacturing method for the manufacture of inner-shield materials, comprising the steps of:

cold-rolling a hot-band steel sheet or strip,

annealing said cold-rolled steel sheet or strip at 550° C.–680° C.,

cold-rolling again the annealed sheet or strip to produce a surface roughness of 0.2–2.0 μm Ra,

electro-depositing a nickel layer with a thickness of 0.1–5.0 μm at least on one side of the steel sheet or strip to provide a surface-treated sheet or strip, and

re-annealing the surface-treated and cold-rolled steel sheet or strip; and

inserting the re-annealed steel sheet or strip into a cathode ray tube for magnetic shielding.

3. A manufacturing method used for the manufacture of inner-shield materials of a color cathode ray tube, comprising the steps of:

cold-rolling a steel sheet or strip;

skin pass rolling said cold-rolled steel sheet or strip to produce a surface roughness of 0.2–20 μm Ra;

electro-depositing a nickel layer with a thickness of 0.1–5.0 μm at least on one side of said steel sheet or strip; and

annealing and recrystallizing said surface-treated steel sheet or strip to provide crystal grain growth and enhanced magnetic shielding characteristics; and

inserting said annealed and recrystallized steel sheet or strip into the cathode ray tube for magnetic shielding.

15

30

35

55

\* \* \* \* \*

60

65

UNITED STATES PATENT AND TRADEMARK OFFICE  
**CERTIFICATE OF CORRECTION**

PATENT NO. : 5,618,401  
DATED : Apr. 8, 1997  
INVENTOR(S) : Nomura et al.

It is certified that error appears in the above-identified patent and that said Letters Patent is hereby corrected as shown below:

Column 4, line 24, delete "titanic" and insert therefor  
--titanium--.

Column 5, line 30, delete "small" and insert therefor  
--smaller--.

Column 8, line 35, delete "prevent of" and insert  
therefor --prevents--.

Column 9, line 45 (claim 3.), delete "0.2-20 and insert  
therefor --0.2-2.0--.

Signed and Sealed this

Thirty-first Day of March, 1998

Attest:



BRUCE LEHMAN

Attesting Officer

Commissioner of Patents and Trademarks